

July 13, 1948.

F. H. VERHOEK ET AL

2,445,253

METHOD OF PRODUCING MIRRORS BY CHEMICAL DEPOSITION

Filed Feb. 6, 1946

2 Sheets-Sheet 1



Fig. 1



Fig. 2



Fig. 3



Fig. 4



Fig. 5



Fig. 6

INVENTORS

Frank H. Verhoek.  
Willard L. Morgan.

*Corbett, Mahoney & Miller*

ATTORNEYS

July 13, 1948.

F. H. VERHOEK ET AL

2,445,253

METHOD OF PRODUCING MIRRORS BY CHEMICAL DEPOSITION

Filed Feb. 6, 1946

2 Sheets-Sheet 2



Fig. 7



Fig. 8



Fig. 9



Fig. 10

INVENTORS  
Frank H. Verhoek  
Willard L. Morgan.

BY  
Corbett, Mahoney & Miller  
ATTORNEYS

## UNITED STATES PATENT OFFICE

2,445,253

METHOD OF PRODUCING MIRRORS BY  
CHEMICAL DEPOSITION

Frank H. Verhoek, Worthington, Ohio, and  
Willard L. Morgan, Haverford, Pa., assignors  
to Libbey-Owens-Ford Glass Company, Toledo,  
Ohio, a corporation of Ohio

Application February 6, 1946, Serial No. 645,940

9 Claims. (Cl. 117—6)

1

This invention relates to a method of producing mirrors by chemical deposition. It is concerned more particularly with and comprises a method and means for restricting the deposition of such mirror deposits to the surfaces which it is desired to coat, while protecting the other surfaces from such deposition by protecting them with a temporary coating of a water-containing inorganic gelatinous coating which may be of various natures and which may, after the mirroring operation is completed, be removed readily.

Chemically deposited mirror reflective coatings upon articles are formed by contacting those surfaces which are to be coated with mirror deposit, with freshly mixed chemical mirroring solutions which react and deposit thereupon a mirror reflective deposit of silver, copper, gold, or lead sulphide, depending upon the solutions employed. In the forming of flat mirrors from glass, plastic, or polished metal sheets it is customary to support these sheets in a horizontal position either upon a cloth covered table or upon a conveyor and to pour the mirroring solution over the top surface of the sheets, upon which surface the mirror deposit is then formed as desired.

Another way of producing such flat mirrors is to support the sheets upon racks in nearly or substantially a vertical position and to spray mirroring solutions against the front surface upon which it is desired to form the highly reflective deposit. In the various methods thus used in producing mirrors, however, in addition to forming the mirror upon the desired treated surfaces, some scattered mirror deposit in streaks and spots is almost invariably formed upon the other side of the sheet as the aqueous solutions overflow onto, or creep around to such other side. As this other side becomes the front side of the mirror when ordinarily used as a second surface mirror, such undesired deposit must be cleaned off in order to place the mirror into useful and saleable condition. In addition to necessitating this extra operation, considerable additional mirror manufacturing cost is involved because of the difficulty of removing these unwanted and objectionable deposits without scratching the mirror deposit, or without at the same time, affecting or destroying to some degree the desired and previously deposited mirror reflective layer which is chemically similar. Thus, many mirrors of original good and saleable quality have to be scrapped due to the damage done during such cleaning operations.

Attempts have been made to prevent the mirroring solutions from forming deposits upon the

2

surfaces other than those desired to be mirrored, by painting, lacquering, or waxing these surfaces; however, the subsequent removal of such coatings by solvents, scraping, and other cleaning methods, have been unsuccessful because of the difficulty of removing such hard coatings and the considerable amount of labor involved. The use of rubber dams applied to the edges of the sheets has also been tried so as to restrict the liquids to the side to be coated but the application of these and their subsequent removal from the wet and slippery glass, or other sheets, presents hazards. Moreover, their use also prevents the edges of the glass, et cetera, from being placed into initial satisfactory clean condition.

One of the objects of the present invention is to provide a new and novel method by which the chemical deposition of a mirror reflective coating or deposit from a mirroring solution may be restricted to only those surfaces which it is desired to coat.

Another object of the present invention is the provision of a new and novel method of mirroring or silvering flat glass, or other sheets of polished material upon the back or top surface, by pouring a chemically reacting depositing solution upon such top surface and by also pre-treating the under surface of the flat glass or other sheet so that no mirror deposit forms thereon.

It is a further object of this invention to provide means for preventing the deposit of mirror reflective materials by means of chemical deposition which can be simply removed in water after the mirroring operation has been completed.

In general, the present invention is preferably carried out by bringing the surfaces which are not to be mirrored into substantially complete contact with an aqueous or water-containing gel of an inorganic compound which acts as a barrier to the chemically mirroring solutions and prevents deposition occurring at such protected surfaces by preventing access of the solutions to the same. As such, it operates with any of the chemical mirroring solutions when these are applied to the surfaces to be mirror-coated and it is thus applicable in the deposition of silver, platinum, copper, gold, or lead sulphide mirrors upon glass, or other supports, while these are supported upon tables or conveyers, or while being mirrored by spraying and while supported in vertical or substantially vertical position. After the mirror deposition, the water-containing gelatinous coating, which is relatively soft, is then removed from the glass or other mirror support body quite easily

by the application of a stream of water, or by light rubbing in water to expose the non-mirrored surfaces thus protected during the mirroring operation and to finish the mirror production directly into a saleable article.

I have found that various water-containing soft gels of metallic compounds may be utilized to secure the desired results of this invention and have employed as such many inorganic metallic compounds which may be formed into water-containing gelatinous coatings, such as silicic acid, titanic acid, many metallic silicates, and numerous metallic hydroxides, certain metallic ferrocyanides, and a few of the metallic sulphides, phosphates, borates, and tungstates. In addition to the satisfactory materials being capable of giving gelatinous water-containing gels for coating use, they must also be water insoluble, as well as being insoluble in the alkaline mirroring solutions to be employed. Thus specifically among the many inorganic metallic compounds which form gels with water, such that they are useful as barriers to the mirroring solutions, and which are not affected by the mirroring solutions, and which I have employed of the above classes, I list the following which are representative, although it will be apparent that there are many others of these types of compounds equally useful: I may use gelatinous coatings of the metallic hydroxides, such as ferrous or ferric hydroxide, copper hydroxide, antimony hydroxide, nickel hydroxide, cobalt hydroxide, cadmium hydroxide, and bismuth hydroxide. The silicates of these same metals are equally useful such, for example, as copper silicate, iron silicate, etc., as are also copper ferrocyanide, zinc ferrocyanide, and iron ferrocyanide. Iron sulphide, copper sulphide and zinc sulphide, as well as iron or barium ortho phosphate, or cadmium, or barium pyrophosphate, may each serve my purposes as a barrier to mirroring solutions; and I may also use silver or copper borate, or iron, or copper tungstate. The various gelatinous compounds may be formed by the interaction of aqueous solutions of two different inorganic compounds selected to provide the necessary final elements, as will be more apparent from the examples below. Thus, to form a ferrocyanide, a soluble alkali ferrocyanide such as potassium ferrocyanide, may be reacted with a soluble metallic salt, such as copper acetate, to form upon contact of the two aqueous solutions, a metallic ferrocyanide water-containing gel or specifically, such a gel of copper ferrocyanide. The solutions may be partly alcoholic and the concentrations of the reactants is not particularly critical provided they are of sufficient strength to form sufficient gel substance that the latter will have a soft body and be coherent.

The gelatinous coating preferably may be applied to or formed upon a face or faces of the support, for example, such as the glass, plastic, or polished metal employed in the forming or manufacture of mirrors, the face or faces which are so coated with the gelatinous coating, being those desired to be kept free of the mirror deposit. However, when working with the ordinary sheet type supports, the production of mirrors may also be carried out by impregnating and covering a cloth mirror table top blanket, or a cloth conveyor belt, with the water-containing gelatinous coating and then placing the face of the sheets, which are to remain unmirrored, directly in contact with these wet gelatinous coatings which immediately substantially contact the

entire surface of the sheet and protect it from the mirroring solutions that are afterwards applied to the upper surface to form a mirror deposit thereon.

5 The foregoing and other objects and advantages of my invention, and various methods of applying the gelatinous coatings; or of forming such coatings either upon the supports of glass, plastic, or other materials to be made into a mirror; or upon 10 the cloths upon which these articles or sheets of materials are supported during mirror formation, will be apparent from the following description, appended claims and the accompanying drawings, wherein like reference characters designate corresponding parts in the several views.

In said drawings:

Fig. 1 is a vertical sectional view of a suitable cleaned support, such as glass, upon which a mirrored or reflective surface may be formed in accordance with the present invention.

Fig. 2 is a transverse vertical sectional view through a suitable apparatus which may be employed for applying a solution of an inorganic material to one side of the support shown in Fig. 25 1.

Fig. 3 is a view similar to Fig. 1 and showing the support of Fig. 1 after having been coated with a solution by the apparatus of Fig. 2.

Fig. 4 is a view similar to Fig. 2 showing the application to the previously coated support, of a second coating or film of a liquid solution which chemically interacts with the previously applied coating.

Fig. 5 is a view similar to Fig. 3 and showing the support after having been coated upon the one face by the apparatus of Figs. 2 and 4 successively with a coating or film of each of two liquid solutions which by chemical interaction have formed a water-containing gelatinous coating of an inorganic compound upon the so treated support.

Fig. 6 is a vertical sectional view of the coated support of Fig. 5 and illustrating the step of applying a reflective coating to the previously uncoated face or surface of said support.

Fig. 7 is a transverse vertical sectional view, partly in elevation, showing one manner or mode of applying a reflective coating to the uncoated surface or face of a support, in which the opposite surface or face of the support is covered with a protective coating and rests flatwise upon a table, conveyer, or other supporting medium.

Fig. 8 is a vertical sectional view of the support or article shown in Fig. 7, after the application of the reflective surface coating or mirror deposit to one face thereof.

Fig. 9 is a view similar to Fig. 8 showing the article after the removal of the protective coating or covering from the first surface or face of the article; and

Fig. 10 is a vertical longitudinal section, partly in elevation, of suitable mechanism or apparatus for supporting and transporting articles to be mirror-surfaced or coated in accordance with the invention.

Before explaining in detail the present invention it is to be understood that the invention is not limited in its application to the details of construction and arrangement of parts illustrated 70 in the accompanying drawings, since the invention is capable of other embodiments and of being practiced or carried out in various ways. It is to be understood also that the phraseology or terminology employed herein is for the purpose 75 of description and not of limitation, and it is

not intended to limit the invention herein claimed beyond the requirements of the prior art.

Referring now to the drawings, wherein suitable apparatus or equipment for performing or carrying out the method of the present invention is shown, together with representative products resulting from practicing said method, a piece of suitable support material such, for example, as glass, is shown as a whole at 11 in Fig. 1. In accordance with my invention, the support 11 is to be provided, preferably, with a reflective or mirrored coating on one face thereof and since it is undesirable to have any of this coating material settle or lodge upon the opposite face of the support, said opposite face is preferably protected by some suitable coating, film, or covering of a suitable material or solution which will not be attacked or penetrated by the reflective or mirror coating material. As seen in Fig. 2, a suitable roller R is disposed within an open top container or pot P containing a solution of an inorganic material, indicated at C. It will be understood that the roller R, as shown, which dips into the solution C, has its peripheral surface coated or covered with a layer or film c of said solution which is transferred to the under face of the glass piece 11 as said piece is moved in the direction of the arrow A to produce a coating layer 12 thereupon, see also Fig. 3.

After the layer or relatively thin film 12 has been applied to one face of the support 11, the coated support as seen in Fig. 3 is then moved over and into contact with the coated peripheral surface of a second and similar roller R' and is provided with a second coating or film of a liquid solution of a second substance which is picked up by roller R' located in a similar receptacle or pot P'. This coating or film c' of the second substance C', by chemical interaction with the first applied substance C, forms a gelatinous coating or covering for the support, as shown at 13, Figs. 4 and 5.

The product thus far completed in accordance with my present method, is shown in Fig. 5, wherein 11 represents the support or support material as a whole and which has been coated upon one of its faces with a coating or film of each of the two liquid solutions C and C' which, by chemical interaction, have combined to form a water-containing gelatinous coating of an inorganic compound upon the support, as seen at 13.

After the protective coating 13 has been applied to one face or surface of the support 11 as explained above, or in any suitable or convenient manner, the support is preferably placed in a vertical position with its uncoated face or surface 11a, see Fig. 6, disposed toward a mixing spray head or nozzle 14. The head is preferably supplied through pipes 14a and 14b, with suitable mirror-forming solutions which combine and are discharged as one solution by the nozzle. The nozzle sprays or deposits the fresh reacting and combined mirror solutions upon the clean face 11a to form a mirror or reflective surface coating or layer 15 thereupon. While the support 11 is shown in vertical or upright position, it is to be understood that it may be disposed in other suitable position, it being also understood that the position or location of the nozzle 14 would be changed or shifted accordingly. Moreover, it is to be understood that to complete the product from the illustrated step of Fig. 6, it is merely necessary to remove the temporary protective film 13.

In accordance with a somewhat modified method embodying the present invention, a support body, such as the glass piece or plate 11, having a protective coating or backing layer 13, as seen in Fig. 7, may be placed upon a plane surface, such as the top 16 of a mirroring table, which top may have a suitable surface covering of fabric 17. When in position as seen in Fig. 7, the top clean face or surface of the support 11 which, of course, has not been covered by the gelatinous coating solution or substance 13, may have applied to it a freshly mixed reacting chemical mirroring solution M to form a mirror surface or layer 18 upon said clean face or surface. The solution may be applied in any suitable manner, the flask 19 shown in Fig. 7 being merely illustrative of one manner or mode of supplying the reflective or mirror covering or coating 18 to the support.

In Fig. 8 the support body 11 is shown after its removal from the mirroring table 16, it being clear that none of the mirroring solution 18 has penetrated the protective layer or covering 13.

In Fig. 9 the final mirror product is shown, the protective coating or covering 13 having been removed to reveal a clean face or first surface.

If it is desired to produce mirrors or reflectors in accordance with my method on a high production basis, the method may be carried out by suitable apparatus which may include an endless belt or conveyer for moving uncoated articles to a mirror-surface-applying station for producing upon the exposed faces or surfaces of the supports, mirrored surfaces, while the opposite faces or surfaces of the supports are protected from being contaminated by the mirroring solution during its application to said exposed faces.

One such suitable apparatus as referred to in the preceding paragraph is shown, somewhat diagrammatically, in Fig. 10. In this figure, suitable supporting framework, shown as a whole at 20, carries a pair of rotatable drums 21 and 22, over which a fabric conveyer belt 23 travels. The framework also carries a plurality of supporting rolls 24 disposed beneath the upper course of the belt 23 to support the same. The belt is preferably provided with a water-containing wet gelatinous coating 13, some of which impregnates the belt, the coating 13 of the belt being adapted to be engaged by the under faces or surfaces of the pieces 11 of support material which may be placed upon the conveyer belt in the vicinity of the drum 22. This gelatinous coating 13 is applied to the lower course of the belt adjacent the drum 22 in a well known manner, by means of two pairs of inking rollers 26 and 27 disposed in tanks or receptacles, 28 and 29, respectively. As the belt 23 travels in the direction of the arrows B shown in Fig. 7, the successive pieces or plates of glass 11 are carried beneath the mixing spray head or nozzle 30 to which fresh reacting mirror-forming solutions are supplied through pipes 31 and 32. The nozzle 30 sprays or deposits the combined mirror solutions upon the clean upper faces of the pieces 11 to produce a mirror or reflective surface coating or layer 15 upon each of them, successively.

It may be desirable to clean the conveyer belt 23 as it is traveling through its lower course as seen in Fig. 10. For this purpose, a water spray issuing from a nozzle 33 may be caused to impinge upon the adjacent portions of the belt. As the belt travels past the water spray station, it encounters a pair of squeeze rolls 34 which serve to remove additional material and surplus

water from the fabric belt. The water and the coating solution flow out to a draining system, shown generally at 35.

*Example 1*

A lead sulphide mirror was made by taking a glass piece cut in the shape of an automobile rear view mirror and thoroughly cleaning one side of the same and then first passing the other side over a felt covered roller dipping into a 20% solution of ferrous chloride, or of ferrous acetate. The same side was then passed over a similar roller dipping into a 20% solution of sodium hydroxide which, by reaction with the first solution applied to the glass, gave a deposit and coating upon the glass of the gelatinous ferrous hydroxide. This gel was quite wet and contained a large amount of water but was sufficiently stiff that it did not carry away when put in contact with liquid, but required some force behind the liquid to do so, or required slight rubbing to remove from the glass. In order to make a thicker layer of gel coating upon the glass, it was repeatedly built up by further successive passages over the rollers supplying the ferrous chloride and the sodium hydroxide. When substantially all of one side of the glass was thus coated with the gel by one or more passages over the rollers, the gel coated side was placed downwards upon a mirror table heated to about 98° F. and a freshly mixed solution for forming a lead sulphide mirror was poured upon the upper clean surface. Any solution suitable for this purpose may be used but I mixed, as disclosed in Colbert U. S. Patent No. 1,603,936 and just before pouring upon the glass, one part of a 4% lead acetate solution with four parts of a 2% thiourea solution. After mixing these well, I quickly stirred in one quart of a 6% solution of sodium hydroxide. The solution readily formed a lead sulphide mirror upon the desired upper face of the glass and the ferrous hydroxide gel upon the lower face was insoluble in the mirror forming solution and prevented it from contacting the lower surface, thereby preventing any deposition of mirror upon such surface. After fifteen or more minutes' time had passed to permit the mirror deposition to become completed by reaction of the mirroring solutions, the surplus liquid was drained off the plate of glass by lifting the same and the ferrous hydroxide gelatinous coating was removed by flushing the same off with a stream of water under pressure and also, if desirable, by lightly rubbing the wet surface with a cloth. The glass was further cleaned, drained, and dried and was then a finished mirror.

*Example 2*

Proceeding in a similar manner a sheet of polished glass was cleaned and then scrubbed with dilute tin chloride solution upon one side and then passed successively over rollers in contact with its other side which dipped in 10% ferric chloride and 10% sodium hydroxide or 10% potassium hydroxide, to produce a water-containing wet gelatinous coating of ferric hydroxide upon one side. Other water-soluble ferric salts, such as ferric nitrate or sulphate, may be used and strong ammonia may serve as the alkali in forming the ferric hydroxide gel coatings. The gel coating while wet and containing a large amount of water, was of sufficient stiffness that it would not slide off the coated glass. The glass was placed with the coated side down upon a cold mirror table and silvered upon the upper ex-

posed surface by pouring thereon the following solution: A solution of 1.25% silver nitrate was made up and to 100 cc. of this there was added 3.7 cc. of concentrated ammonia hydroxide to clear the same, and then sufficient sodium hydroxide to make the latter equal to 1.0% of the mixture. With one part of this mixture there was mixed quickly, one part of a 5% invert sugar solution. The mixture thus produced was promptly poured upon the glass, where it deposited a silver mirror coating but as the ferric hydroxide gelatinous coating was completely unaffected by these mirroring solutions, no silver deposition occurred on the gel-coated and protected face of the mirror. The gel was then removed by ordinary washing and the glass, after drying, was a completed mirror entirely free of undesirable mirror spots or stains upon its face.

In a similar manner the ferric hydroxide gel-coated glass piece may have been made into a gold mirror by the placing of the same upon the mirror table and the pouring upon the uncoated exposed surface of a gold mirroring solution, such as mixtures of alkaline gold chloride solution and formaldehyde solution, commonly used for gold mirror deposition. The alkaline formaldehyde solutions do not affect the gel coating and it amply protects the surface which is to be kept clear from any mirror deposition.

*Example 3*

A clear glass-like sheet of Columbia resin plastic such as manufactured by the Pittsburgh Plate Glass Company which is presumably a polymerized allyl methacrylate resin, was steeped for fifteen minutes in a 5% solution of sodium hydroxide, rinsed, carefully cleaned upon one side, treated in a dilute solution of stannous chloride upon the same side, and then rinsed. The other side was then coated with a copper hydroxide water-containing soft gel by passing the latter face over a felt covered roller which applied to the resin a thin film of copper acetate solution of 10%, 20%, or stronger strength. The treated face was then passed over a similar roller which supplied sodium hydroxide solution or potassium hydroxide solution of 5% or greater strength. The strength of the solution is relatively immaterial. Each could be and was adjusted so as to produce upon the surface treated, a gelatinous coating of sufficient stiffness, or body, that it did not slide off of the treated surface and substantially covered the entire surface treated.

The plastic sheet was then placed upon a mirror table and a silver mirror was deposited upon the exposed surface by the application of the silvering solution described in Example 2, above. The copper hydroxide gel was washed off after the silvering operation to give a plastic silver mirror free of mirror deposit upon its face.

In the manner set forth in the three examples above, other metallic hydroxides may be formed by reaction of metallic salts which are water soluble with the alkaline water-soluble hydroxides, sodium hydroxide, potassium hydroxide, ammonium hydroxide, or lithium hydroxide. Mirroring solutions for chemical deposition of silver, platinum, gold, copper, and lead sulphide, which comprise the materials which may be deposited from water solutions as mirror deposits, are all alkaline solutions and may contain in the various formulae known in the mirror art, either sodium hydroxide or equivalent potassium hydroxide, or may contain one of these in combination with ammonium hydroxide. The latter is

generally present in small quantity and, provided a metallic hydroxide gel is chosen and which is insoluble in excess sodium or potassium hydroxides, and which may be formed into a gelatinous coating, the choice of metallic hydroxides which are useful in the forming of mirrors by the methods embodying the present invention, is broad, and many materials of this type can be used quite satisfactorily. In the last example, it is to be pointed out that the copper hydroxide gelatinous coating employed, while soluble in strong ammonia, was unaffected by the small amount of ammonia present in an ordinary silvering solution. Aluminum hydroxide and zinc hydroxide, which give water-insoluble gels, are not useful, however, because these gels dissolve readily in the caustic alkalies present in the mirroring solutions. While calcium hydroxide is relatively insoluble in water and in the mirroring solutions, it does not give gelatinous precipitates or coatings and it is not useful as a protective barrier against deposition of the mirror deposits. I may use gelatinous coatings of the metallic hydroxides of bismuth, cadmium, cobalt, nickel, antimony, copper, iron and others which are insoluble in excess of the strong alkalies, and insoluble in the mirroring solutions.

In a similar manner I have found that the metallic silicates of the same metals are insoluble in the mirroring solutions and that they readily give water-containing gelatinous coatings which act as effective barriers to such solutions and that they may be employed as coatings to protect surfaces of glass, or other support articles, during the mirroring of other surfaces.

#### Example 4

The fabric belt of a continuous conveyer used in the production of mirrors in an apparatus or machine of the type represented in Figure 10 of the accompanying drawings, was impregnated as shown in that figure, by passing the belt over an inking roller of a pair supplied with a 10% or stronger solution of any of the available commercial grades of the alkali sodium or potassium silicate solutions in water and then run over a second roller of another pair which carried a 10% or stronger solution of ferrous chloride which, by reaction with the soluble silicate, gave a heavy wet gelatinous coating on and impregnation of the fabric belt, of ferrous silicate. As the belt passed around the drum at the head of the conveyer (at the right side of Fig. 10) a cleaned piece of glass was laid upon the conveyer directly upon the soft gelatinous coating upon the fabric and the latter wet coating immediately contacted the face of the glass and sealed it at the edges so that when the subsequent mirroring solution for forming a mirror was applied to the top of the glass as it traveled along with the conveyer belt, it did not run under the glass and did not contact, in any way, the lower surface of the glass, the mirror deposition being restricted to the desired top surface only. When a lead sulphide mirror was to be formed, the same solutions as were employed in Example No. 1 were employed, the glass being preferably slightly heated as it passed along the conveyer prior to the application of the mirroring solution. When a silver solution, such as that given in Example No. 2 was employed, a silver mirror was so produced. At the end of the conveyer, the mirrored glasses were removed and by a simple washing, any adhering particles of gelatinous coating were readily removed and after drying,

the mirror was complete. As a further example of suitable siliceous compounds in addition to the metallic silicates, I may use silicate acid, as shown in the next example.

#### Example 5

In a similar continuous conveyer mirroring apparatus or machine, the first pair of inking rollers was fed with an alkali silicate solution as before, but the second pair of rollers was rotated in a bath of, and thus fed with a solution of 5%, or stronger, of an acid, such as hydrochloric acid, sulphuric acid, or sodium bisulphate which, by reaction with the silicate solution, formed a coating upon and an impregnation of the fabric, of a wet water-containing gel of silicic acid. Such gel does not readily go into solution again in the alkali solutions used in mirroring, such as the lead sulphide mirror forming solutions and the silvering solutions given in the above examples. Moreover, it is also resistant to solution action by mirroring solutions containing tartrates as are used in some silvering formulae and to the phenylhydrazine or formaldehyde appearing in the alkaline solutions for the forming of copper mirrors. After the application of any of these mirroring solutions upon glass laid in the gel coating upon the fabric belt and the formation of a mirror deposit upon the unprotected side, the glass was removed from the end of the conveyer (at the left side of Fig. 10) and the attached gel readily washed off with water. Thus, the faces of the second surface mirrors so produced were found to be clean and entirely free of the mirror deposit.

#### Example 6

A gelatinous protective coating of precipitated titanic acid presents the same useful advantages found with silicic acid coatings. A cleaned piece of glass was coated upon one side with such a water-containing wet gel coating of titanic acid, by passing the surface of the glass which it was desired to keep clear, over a roller supplied with a strong solution of titanium sulphate and then over a second roller carrying sodium hydroxide solution. Upon subsequently applying a mirroring solution to the uncoated surface, such as by holding the glass in a vertical rack and spraying a silvering solution, such as that given in Example No. 2, or other silvering solution, such as those known in the art employing phenyl-hydrazine, onto the uncoated surface, it was found that although considerable of the mirroring solution splashed directly upon the back of the glass, the gelatinous coating completely protected the glass from receiving any mirror deposit upon such surface. Upon the subsequent removal of the gelatinous coating by a stream of water under pressure, the mirror coating was found to be entirely restricted to the desired back surface and the face of the second surface mirror so produced was free of the mirror deposit.

#### Example 7

Where we are forming a lead sulphide mirror we may use a protective water-containing gelatinous coating of a metallic sulphide which is insoluble in the lead sulphide mirroring solution. Thus, the glass or other article to be mirrored, was first cleaned and then passed over a felt roller dipping in a 10% solution of sodium sulphide and then passed over a second such roller carrying a 15% solution of copper nitrate or of 15%, or stronger solution of ferrous ammonium sulphate, so that there was formed upon the surface

so treated, a soft gelatinous coating of copper sulphide, or of ferrous sulfide, respectively. A glass having one surface thus coated was placed upon a warm mirroring table with the gel-coated side down against the table. The mirroring solution as employed in Example 1 was then poured upon the exposed surface and a lead sulphide mirror formed thereon. The plate was then removed from the table and the soft gel washed off in water by light rubbing with a cloth and the entire washed plate was then dried to give a mirror free of any lead sulphide deposit upon the face opposite to that carrying the mirror coating.

*Example 8*

Six pieces of glass were carefully cleaned and then one set of three pieces was scrubbed with a very dilute solution of stannous chloride upon one face, and subsequently rinsed well. These three pieces of glass were then passed over a roller having a felt covering which dipped into a 10% solution of potassium or sodium ferrocyanide, the surface brought into contact with the roller being, in each case, the non-tinned surface. The same surface was then passed over a similar set of rollers to form a metallic ferrocyanide gelatinous water-containing coating thereon. The first piece was passed over a roller fed with a 10% solution of copper chloride and had formed thereon a copper ferrocyanide gelatinous coating. The second piece was passed over a roller fed with 10% zinc sulphate and the latter reacted with the soluble ferrocyanide film to form a gelatinous coating upon the glass, of zinc ferrocyanide. The third piece was passed over a roller carrying a 10% solution of ferric chloride to form ferric ferrocyanide thereon. The second set of three glasses which were not tinned were each, respectively, coated with copper, zinc, or ferric ferrocyanide in the same manner.

Upon the tinned surface of the glass plate carrying a coating upon its other side of copper ferrocyanide, there was poured a freshly mixed silvering solution employing sugar as the reducing agent, such as that employed in Example No. 2 and a silver mirror deposit was thus formed. In similar manner, a silvering solution employing sodium potassium tartrate as the reducing agent and alkali, such as any of the well known Rochelle salt silvering formulae, was poured upon the tinned surface of the glass protected upon its other side by a zinc ferrocyanide gelatinous coating. Upon the third glass, carrying a protective coating of ferric-ferrocyanide upon one side, there was poured on the clean tinned side, a silvering solution employing an alkaline solution of formaldehyde as the reducing agent and a silver mirror deposit was formed. Upon the other three non-tinned glasses, there was poured upon the clean non-coated side of each, a lead sulphide mirror-depositing solution, such as that employed in Example No. 1, to form a lead sulphide mirror, while in each case the other side was protected by a gelatinous coating of metallic ferrocyanide, respectively, copper, zinc, and ferric ferrocyanides with the three glasses.

In each case the ferrocyanide coatings were then removed after the mirror deposition was complete and in every case, there was no mirror deposit found upon the face of the six mirrors produced.

*Example 9*

A cleaned piece of glass was coated with a film of a 20% solution of ferric chloride. Then a so-

lution of 20% sodium tungstate was brought into contact with the film to react with the same and to deposit upon the glass in substantially complete contact therewith, a gelatinous coating of iron tungstate which is insoluble and which, as a coating, was quite wet and obviously carried a lot of water within the gel. The other side was then subjected to a freshly mixed lead sulphide mirroring solution and a lead sulphide mirror deposit formed thereon. Despite the mirroring solution having run over the sides of the glass and thus around to the face protected by the gelatinous coating, there was no mirror coating found upon the thus protected face after the glass was washed in water to remove the gelatinous coating.

We claim:

1. The method of making mirrors by chemical deposition of an alkaline mirroring solution upon one surface of a sheet-like support, which comprises substantially completely contacting one surface of the support with a water-wet gelatinous coating so as to protect said surface from contact with said alkaline mirroring solution to be applied to the other surface of the support, said gelatinous coating consisting of gelatinous water-insoluble inorganic metallic compound material and a sufficient amount of water to form a stiff non-flowable gel that closely adheres to said surface, said coating being insoluble in said alkaline mirroring solution and being sufficiently stiff to prevent displacement by any of such solution which might reach it after being applied to said other support surface, and then applying to said other support surface, while the gelatinous coating is still on said first support surface and is still wet, said alkaline mirroring solution and depositing a mirror deposit upon such other surface.
2. A method according to claim 1 wherein the gelatinous coating is removed after completion of the mirroring deposit by means of an aqueous treatment with gel displacing pressure which exposes the non-mirrored surface of said support.
3. A method according to claim 2 wherein the coating is gelatinous water-insoluble metallic hydroxide.
4. A method according to claim 3 wherein the coating is gelatinous water-insoluble iron hydroxide.
5. A method according to claim 2 wherein the coating is gelatinous water-insoluble metallic sulphide.
6. A method according to claim 2 wherein the coating is gelatinous water-insoluble metallic ferrocyanide.
7. A method according to claim 3 wherein the coating of gelatinous water-insoluble metallic hydroxide is produced by reacting in place on said surface of the support to be protected an aqueous solution of water-soluble alkali hydroxide and an aqueous solution of metallic salt that will react with the said alkali solution to form a water-insoluble metallic hydroxide water-containing gel.
8. A method according to claim 5 wherein the coating of gelatinous water-insoluble metallic sulphide is produced by reacting in place on said surface of the support to be protected an aqueous solution of water-soluble alkali sulphide and an aqueous solution of metallic salt that will react with the said alkali solution to form a water-insoluble metallic sulphide water-containing gel.
9. A method according to claim 6 wherein the coating of gelatinous water-insoluble metallic ferrocyanide is produced by reacting in place on

**13**

said surface of the support to be protected an aqueous solution of water-soluble alkali ferrocyanide and an aqueous solution of metallic salt that will react with the said alkali solution to form a water-insoluble metallic ferrocyanide water-containing gel.

FRANK H. VERHOEK.  
WILLARD L. MORGAN.

**14****REFERENCES CITED**

The following references are of record in the file of this patent:

5

**UNITED STATES PATENTS**

| Number    | Name       | Date          |
|-----------|------------|---------------|
| 1,042,827 | Schumacher | Oct. 29, 1912 |
| 2,317,877 | Ballantine | Apr. 27, 1943 |

**Certificate of Correction**

Patent No. 2,445,253.

July 13, 1948.

**FRANK H. VERHOEK ET AL.**

It is hereby certified that errors appear in the printed specification of the above numbered patent requiring correction as follows: Column 7, line 39, Example 1, for the word "quart" read *part*; column 8, line 48, Example 3, for "solution" read *solutions*; column 10, line 3, Example 4, for "silicate acid" read *silicic acid*; and that the said Letters Patent should be read with these corrections therein that the same may conform to the record of the case in the Patent Office.

Signed and sealed this 12th day of October, A. D. 1948.

**[SEAL]**

**THOMAS F. MURPHY,**  
*Assistant Commissioner of Patents.*